

Jan. 15, 1935.

A. J. MASON

1,988,387

## PRODUCTION OF PHOSPHORUS

Filed Aug. 27, 1930

6 Sheets-Sheet 1



Inventor:  
Arthur J. Mason,  
By Dunnington, Jr., Chittenden & Miles,  
Attorneys.

Jan. 15, 1935.

A. J. MASON

1,988,387

## PRODUCTION OF PHOSPHORUS

Filed Aug. 27, 1930

6 Sheets-Sheet 2



*Inventor:*

Arthur J. Mason

By Dyerforth, Lee, Chitton, & Hills  
A. T. B. S.

Jan. 15, 1935.

A. J. MASON

1,988,387

PRODUCTION OF PHOSPHORUS

Filed Aug. 27, 1930

6 Sheets-Sheet 3



Inventor:  
Arthur J. Mason,  
By Dyerforth, Lee, Critton & Willis,  
Attejs

Jan. 15, 1935.

A. J. MASON

1,988,387

PRODUCTION OF PHOSPHORUS

Filed Aug. 27, 1930

6 Sheets-Sheet 4



Inventor:  
Arthur J. Mason,  
By Dyerforth, Lee, Chittenden & Niles,  
Attys.

Jan. 15, 1935.

A. J. MASON

1,988,387

PRODUCTION OF PHOSPHORUS

Filed Aug. 27, 1930

6 Sheets-Sheet 5



Inventor:  
Arthur J. Mason,  
By Dyrnforth, Le, Chittenden & Niles,  
Atty.

Jan. 15, 1935.

A. J. MASON

1,988,387

PRODUCTION OF PHOSPHORUS

Filed Aug. 27, 1930

6 Sheets-Sheet 6

Fig. 11.



Fig. 10.



Inventor:  
Arthur J. Mason,  
By Dymforth Lee, Chritton & Miles,  
Attest.

## UNITED STATES PATENT OFFICE

1,988,387

## PRODUCTION OF PHOSPHORUS

Arthur J. Mason, Homewood, Ill.; Continental Illinois National Bank and Trust Company of Chicago, executor of estate of said Arthur J. Mason, deceased

Application August 27, 1930, Serial No. 478,194

3 Claims. (Cl. 23—223)

The present invention relates to improvements in the recovery of the phosphate values of mineral phosphates in the form of phosphorus or compounds thereof, such as phosphoric acid or phosphorus pentoxide, and more particularly to such processes wherein the phosphorus content of the mineral is reduced and volatilized by the use of a suitable carbonaceous material.

Volatilization processes for the recovery of the phosphorus values from phosphates have hitherto been attended with many serious disadvantages. In such processes, of which the blast furnace type of operation is typical, high temperatures of operation are required, and the attainment of such temperatures can be secured effectively only by the combustion of the fuel employed with a reasonable efficiency so as to produce substantial amounts of carbon dioxide. This carbon dioxide, in the quantities present, in turn serves as an oxidizing agent for the carbonaceous material present in the reaction zone in which the reduction of the phosphate of the mineral is to be effected and consequently necessitates the introduction of excessive quantities of the reducing agent and lowers the efficiency of the reducing operation.

Furthermore, in such processes, as hitherto conducted, large volumes of gases must be forced through and in contact with the reaction mixture, and these gases, which include the gases from oxidation of the fuel and carbonaceous reducing agent used in the process, must be subsequently handled for the recovery of the phosphorus contents thereof, for example, in electrostatic precipitators. The handling of the large volumes of gases at high velocities introduces fume and dust problems, reduces the efficiency of recovery of the phosphorus values, and greatly increases the cost of recovery. It likewise makes impractical the employment of the ordinary rotary kiln-type of furnace, the use of which would be highly desirable from the standpoint of efficiency and economy.

The high temperatures employed in such volatilization processes as hitherto proposed for practical use, and required for the fusion of the slag and ferrous constituents of the reaction mixture, have the further disadvantage of inducing a considerable loss of phosphorus by reaction with iron and other metallic constituents of the mixture with the formation of the corresponding phosphides, such as ferrophosphorus. Thus ferrophosphorus containing as high as 25 to 30% of the phosphorus may be formed as a by-product of such processes.

The present invention has as its object a reduction process for the recovery and removal of the phosphorus values of a phosphorus-containing mineral, employing carbonaceous material as reducing agent and as fuel, which is not attended with the disadvantages of such processes as hitherto carried out. As an important feature of the invention, I separate the time periods of heating the furnace employed and of heating the phosphatic charge therein. I prefer to employ as the furnace a refractory-walled chamber, and while it may be exteriorly heated, I prefer to heat it interiorly by the application of hot gases or by interior combustion of fuel gases or preferably of phosphorus-containing gases resulting from the phosphate reduction operation. A sufficient heat is stored in the walls of the chamber, heating thereof is then stopped, and the phosphatic charge introduced and reduction and volatilization of the phosphorus effected. In this reduction and volatilization, heat is absorbed from the walls of the reaction chamber and after discharge of the spent reaction mixture, the reaction chamber is again heated and the operation repeated. I prefer to utilize a system containing two or more reaction chambers, the gases evolved in one during the reduction and volatilization process being burned in another to convert their phosphorus content into phosphorus pentoxide and at the same time to supply the necessary heat for its interior walls to bring it to the necessary temperature for conducting in it a reduction and volatilization operation upon another charge.

In operating in accordance with my invention, the reduction and volatilization is effected in a substantially quiescent atmosphere, preferably of a reducing character and consisting largely of carbon monoxide, and without passage through the charge of the large volumes of combustion gases or dilution of the phosphorus therewith, as in fuel-fired volatilization operations hitherto commercially employed. I prefer to conduct the operation without fusion of the reaction mixture, and thereby avoid the necessity of incorporating into the charge large proportions of fluxes or slag-forming constituents and prevent the combination of phosphorus with the metallic constituents of the charge, such as iron, to a very great extent. By preparing the charge as herein set forth, I secure an intimate contact of the phosphate rock in the finely divided, incandescent carbon during reaction and thereby greatly facilitate reduction. In order that the invention may be fully

understood, I have described it hereinafter in connection with certain specific embodiments of apparatus suitable for carrying it into effect, but it will be understood that these details of apparatus and of specific procedure therein are not intended to be regarded as limitations upon the scope of the invention, since obviously numerous other forms of apparatus and other details of procedure may be employed.

10 Figure 1 is a side elevation of apparatus suitable for carrying the invention into effect;

Fig. 2 is a plan view of a portion of the apparatus, showing a pair of reaction furnaces;

15 Fig. 3 is an enlarged elevation, partly in section, of a portion of the preheating or carbonizing furnace; and

Fig. 4 is an enlarged sectional view of another portion, the discharge end, of the pre-heating or carbonizing furnace;

20 Fig. 5 is a vertical sectional view through the reaction furnaces on the line 5 of Fig. 1;

Fig. 6 is a vertical sectional view through a portion of the receiving end of a reaction furnace, on the line 6 of Fig. 2; and

25 Fig. 7 is a vertical sectional view through another portion, the discharge end, of a reaction furnace on the line 7 of Fig. 2;

Fig. 8 is a transverse sectional view on the line 8 of Fig. 6; and

30 Fig. 9 is a transverse sectional view on the line 9 of Fig. 7; and

Figs. 10 and 11 are respectively vertical and horizontal sectional views through an air pre-heater employed in the present invention.

35 In the drawings, the numeral 15 designates a fired furnace setting for a preheating or carbonizing furnace, suitably such as that described in my prior application Serial No. 441,547, filed April 4, 1930. This furnace is provided with an elongated chamber 16, through which pass the combustion gases from the furnace portion 17. A rotatable cylindrical furnace 18 having a downward inclination extends longitudinally through the furnace chamber 16, and is provided at its receiving end with a closure 19 upon which is mounted the drive gear 20. A stationary trunnion 21 passes through the closure member 19, opening into the interior of the rotatable furnace 18, the charge, composed as hereinafter described, being fed through the trunnion 21 by any suitable means, such as the screw 22. The charge is initially delivered to a receiving hopper 23 and is passed successively through chambers 24 and 25, provided with valve closures 26, which may be alternately operated in the customary manner to feed the charge without permitting escape of gases. From the chamber 25, the charge is picked up by the screw 22 to be fed into the furnace 18.

60 At its discharge end, the furnace 18 opens into a receiving chamber 27, suitably with heavy refractory walls to serve as insulation and prevent loss of heat. In the upper portion of the rotating furnace 18, a cutter bar support 28 is provided, being pivotally mounted at one end on a bracket 29 on the trunnion 21 and at the other end on a bracket 30 carried by the wall of the receiving chamber 27, the cutter bar 28 being provided with a tool steel cutter edge 31 extending the length of the rotating furnace 18, and being so mounted that the cutter edge 31 is held in juxtaposition to the wall of the cylindrical chamber 18 on the ascending side thereof, as more fully set forth in my prior application Serial No. 441,547, hereinbefore referred to,

I feed to the preheating and carbonizing furnace 18 a charge consisting of the phosphate mineral and carbonaceous material, preferably bituminous or cooking in character, in suitable proportions for the necessary reactions in the system ranging, for example, from 5 to 10 parts carbonaceous material to 10 parts of phosphate mineral, the materials charged being preferably ground moderately fine, say to about 80 mesh. Thus, I may employ a mixture of about equal proportions of mine-run Tennessee phosphate rock and bituminous coal. Such a charge is fed to the hopper 23, passes through the chambers 24 and 25, and forced into the preheating and carbonizing furnace 18 by means of the screw 22. The furnace 18 is rotated and is heated to a suitable temperature, say 1000 to 1200° F., the carbonaceous material therein is partially or wholly coked, and volatile and liquefied constituents of the coal permeate the mass, resulting in an intimate association of carbonaceous material and finely divided phosphate rock throughout the entire body of material. By the combined action of the rotation of the furnace and of the cutter bar 31, the mixture is agglomerated into small granules or lumps. The gases from the preheating operation together with the agglomerated material pass into the receiving chamber 27, the reaction mixture being then at a temperature of say 900 to 1100° F. and preferably about 1000° F. The gases from the preheating operation are drawn off through the pipe 32 and are utilized in the system as hereinafter set forth.

The hot lumps or granules of reaction mixture pass out of the chamber 27 through an opening controlled by bell valve 33 into a refractory walled chamber 34, and from the latter through an opening controlled by bell valve 35 into a chamber 36 provided with two discharge spouts 37 and 38, controlled by valves 39 and 40 respectively. By the discharge spouts 37 and 38 the reaction mixture may be directed to either of two reaction furnaces 41 and 42, of similar construction. For simplicity, the corresponding parts of these reaction furnaces will be designated by identical numerals.

Each of the reaction furnaces 41 and 42 is formed of a cylindrical body portion 43 of refractory material, provided at one end with a receiving head 44 and at the other end with a discharge head 45, the entire furnace being enclosed by a metallic casing 46. On this casing there are provided the supporting rings 47 carrying the ring-gears 48, the furnace being supported and rotated thereby as is customary with rotating furnaces. The refractory material employed is preferably one having characteristics of high heat conductivity, high specific heat and high density in so far as these are conveniently attainable, so that it will rapidly store up a considerable quantity of heat and readily yield it up. Refractories such as carborundum and magnesite have been found suitable.

The receiving head 44 of each furnace is provided internally with an annular pocket 49 of irregular section, as best shown in Fig. 8, this pocket being formed with an inner cylindrical wall concentric with the axis of the furnace and an outer wall 51 eccentric thereto. In consequence, the pocket 49 has a constricted portion 52, and from this constricted portion a port 53 is provided opening into the cylindrical body 43 of the reaction furnace. At a larger portion thereof, the pocket 49 is provided with a port 54.

extending laterally through the body of the receiving head and closed by a gate 55 in the casing 46, the port 54 and gate 55 being in such a position that, when required, they may be brought in 5 juxtaposition to the opening of one of the spouts 37 or 38, as the case may be, to receive the charge for the furnace.

The discharge head 45 is likewise provided internally with an annular pocket 56, formed with 10 concentric walls. At one point, this pocket is provided with a port 57 extending to the interior of the cylindrical body 43 of the furnace at its lower end, to receive material from the furnace.

At another point, the pocket 56 is provided with 15 a laterally extending port 57, closed by a gate 58 in the casing of the furnace, and through which material may be discharged from the pocket.

In the operation of either furnace, for example, the furnace 41, it is preliminarily heated 20 to bring the interior walls in the effective reaction zone near one end to a temperature substantially above 1200° C. and preferably to 1400 to 1500° C., this preheating being preferably effected by the combustion in the furnace of phosphorus-containing gases derived from another 25 operation or of combustible gases from the preheating and carbonizing operation already described, or both. The preferred manner of this preheating will be hereinafter more fully set forth.

After the interior of the furnace has been suitably preheated, a charge of the reaction mixture of phosphate mineral and the carbonaceous material is introduced into the pocket 49 in the receiving head 44 of the furnace. The preferred 30 reaction mixture is the agglomerated material derived from the preheating and carbonizing operation above set forth and is delivered from the receiving chamber 27 of said furnace through the appropriate delivery spout 37 or 38. When 35 a charge of the material has been placed in the pocket 49 in the receiving head 44 of the furnace, the furnace is rotated, and by its rotation there is a slow and progressive feed of the material from the pocket in the receiving head through 40 the port 63 into the body of the furnace, through which the reaction mixture gradually progresses. As it travels through the furnace, it passes progressively into more highly heated portions of the furnace and is heated to a temperature effective for the reduction and release of the phosphorus content of the mineral, without effecting 45 fusion, such temperature being from 1100 to 1300° C., and preferably about 1200° C. The phosphorus is released from the reaction mixture in an atmosphere almost completely of carbon monoxide, an excess of carbonaceous material being supplied to maintain such an atmosphere, since I have found that at such relatively low, nonfusion temperatures above referred to, in the 50 presence of an atmosphere of carbon monoxide, substantially complete reduction and volatilization of the phosphorus content of the mineral is effected. Under these conditions, there is no appreciable fusion or slagging of the reaction 55 mixture, and the spent reaction mixture is of about the same order of fineness or even finer than the reaction mixture charged. During the period of reaction, the rotating furnace is sealed at its lower end, as hereinafter set forth, and the phosphorus vapors, together with carbon monoxide and any other gases evolved, pass out through an opening 59 provided centrally of the receiving head, for recovery of the phosphorus or for combustion thereof to phosphorus pentoxide, 60

the latter to be recovered as phosphoric acid in the usual manner.

It is apparent that, by carrying out the reaction in this manner, a minimum of extraneous gas is present and a high concentration of phosphorus vapor in the evolved gases is secured. 5

As it reaches the discharge end of the furnace, the spent reaction mixture is discharged progressively from the body of the furnace through the port 57 into the pocket 56, in which 10 it accumulates until the entire charge fed into the receiving head 44 has passed through the furnace and been treated. This charge is so adjusted that the stored heat in the walls of the furnace will effect the desired reaction. When 15 the spent reaction mixture has been completely accumulated in the pocket 56, the furnace is rotated until the gate 58 is lowermost, and the gate is then opened to discharge the spent reaction mixture. Heating may be resumed as soon 20 as the spent charge reaches the pocket 56.

In carrying out the invention, it is preferred to employ a plurality of reaction furnaces, for example, two, as shown in the drawings, and while carrying out the reaction in one of the furnaces, 25 directing the evolved vapors therefrom into another furnace and burning them therein to convert their phosphorus content into phosphorus pentoxide, and at the same time heat such furnace internally to the required temperature for 30 carrying out the reaction. When reaction in the first furnace ceases and the reaction material is discharged, or during the period of its discharge, the reaction mixture having been charged into the second furnace, the reaction is conducted 35 therein and the evolved vapors directed into and burned in the first furnace, in a similar manner. Furthermore, as hereinbefore indicated, the gases evolved from the preheating furnace may be employed during a portion of the operation of 40 preheating the reaction furnace. In the drawings, connections suitable for such purposes are illustrated. Reheating of either furnace may be begun as soon as the charge therein has completed its reaction and during or after discharge 45 of the spent reaction material.

In the lay-out shown in the drawings, and best seen in Fig. 2, it will be assumed that reaction is about to take place in the furnace 41, the furnace 42 having just been emptied of spent 50 reaction mixture and being ready for preheating.

For a short period after the reaction mixture has been fed to the furnace 41, and before the initial portions of it passing through the furnace reach reaction temperatures, there is no evolution of combustible vapors therefrom. During this period, combustible gas from the preheating and carbonizing furnace 15, which is continuously operated, is discharged through the pipe 32 and enters a conduit 60, from which 55 a valved branch line 61 leads to a trunnion 62, which passes centrally through the discharge head 45 of the furnace 42. Air for the combustion of this gas is delivered by a pump 64, by which it is forced through an air preheating furnace 65, being discharged therefrom through the hot air-line 66, from which a valved branch 60 leads to the trunnion 62.

As soon as the evolution of the phosphorus-containing combustible gas from the furnace 41 begins, the hydrocarbon fuel gas from the carbonizing furnace 15 is diverted and provision is made for the introduction of the phosphorus-containing gas into the discharge end of the furnace 42. When such diversion is to be effected, 75

the valved line 62 from the gas conduit 61 is closed, and this gas is diverted to a manifold 67, from which it passes through the valved lines 68 and 69 to the burners 70 and 71 of the air preheating furnace 65, air for these burners being supplied through the valved lines 72. Combustion of the hydrocarbon fuel gas from the carbonizing furnace 17 is then continued in the air preheating furnace 65, the air passing through a coil 73 provided therein, until the hydrocarbon gas is required in the initial stages of preheating of the furnace 41, when it is diverted for that purpose, as hereinafter set forth.

The hydrocarbon gas no longer passing to the furnace 42, the phosphorus-containing gas which is evolved from the furnace 41 and passes out of the latter through a trunnion 74 at its receiving end, is caused to flow through a valved connection 75 to a conduit 76. A second valve connection 77 to the trunnion 77<sup>a</sup> is closed at this time, its function being hereinafter set forth.

From the conduit 76, the phosphorus-containing gas passes through a valved connection 78 to the trunnion 63, being mixed with the preheated air which is still being supplied through the valved connection 67. The phosphorus-containing gas is burned in the furnace 42, bringing it to the desired operating temperature, preferably around 1400 to 1500° C. near its discharge end, where combustion takes place, the temperature being lower at the receiving end which serves as a preheating zone utilizing the heat of the combustion gases as they travel through the furnace. The temperature at the receiving end of the furnace will ordinarily be 600 to 700° C. The burned vapors and gases from the furnace 42 during the entire preheating period pass out through the trunnion 74<sup>a</sup>, which is provided with two valve connections. The valve connection 75<sup>a</sup>, which corresponds to the connection 75 on the furnace 41, is closed and the valve connection 77<sup>a</sup> is open. The connection 77 is provided with two branches. During the period of combustion of the hydrocarbon gas from the preheating and carbonizing furnace 15 in the reaction furnace 42, the connection 78 is opened, to permit discharge of the combustion gases to the stack. When the hydrocarbon gases are diverted from the reaction furnace 42 and combustion of phosphorus-containing gas begins therein, the connection 78 is closed and the connection 79 opened, the latter leading to suitable scrubbing and precipitating devices for removing phosphorus pentoxide or phosphoric acid from the gases.

When the reaction in the furnace 41 is completed, at which time the furnace 42 has been preheated to the desired temperature, rotation of the furnace 41 is stopped for the discharge of the spent reaction mixture as hereinbefore described, the connection 75 to the trunnion 74 for discharge of phosphorus-containing vapors having been closed. At the same time, the valve connections 67 and 78 to the trunnion 63 of furnace 42 are closed, and the latter is charged with a batch of reaction mixture, which is caused to travel through the furnace, gradually attaining reaction temperature. Operation of furnace 42 is then started for the conduct of the reaction. The furnace 41 is preheated in a manner similar to that described in connection with the preheating of furnace 42. The air connection 67<sup>a</sup> and the gas connection 62<sup>a</sup> from the gas conduit 61, both leading to the trunnion 63<sup>a</sup>

at the discharge end of furnace 41 are opened, the combustible mixture ignited within the furnace and its burning continued until phosphorus vapors are evolved from the furnace 42. At this time, the gas connection 62<sup>a</sup> is closed, the gas being diverted to the burners and air preheater 65 as above described, and the phosphorus vapor connection 75<sup>a</sup> from the trunnion 74<sup>a</sup> of furnace 42 is opened. The connection 75 from the trunnion 74 of the furnace 41 is closed at this time, and the phosphorus vapors from the furnace 42 pass out through the connection 75<sup>a</sup>, the phosphorus conduit 76, and are directed through the connection 78<sup>a</sup> to the trunnion 63<sup>a</sup> of furnace 41. During the preheating period in the furnace 41, the connection 77<sup>a</sup>, the trunnion 74 is opened, leading through connection 79<sup>a</sup> to the stack during the period in which gas from the carbonizing and preheating furnace 15 is burned in the furnace 41 and through the connection 80<sup>a</sup> to the phosphoric acid scrubbers and precipitators during the period in which phosphorus-containing vapors are being burned in the furnace 41.

In this manner, reaction is caused to take place alternately in the furnaces 41 and 42, and during reaction in either, the other is preheated to the necessary temperature, preferably by combustion therein of the gases evolved from the furnace in which reaction is taking place. Although specifically described in connection with a lay-out containing two furnaces, it is readily apparent that additional furnaces may be employed, with proper control of the reaction and preheating periods therein with respect to one another.

I claim:

1. In the art of producing phosphorus, heating a reaction mixture of phosphate and reducing agent in a reaction chamber, thereby evolving phosphorus-containing vapor therefrom, conducting said phosphorus-containing vapor into a second reaction chamber and burning it therein, internally heating the walls of the second reaction chamber, and on termination of the reaction and evolution of phosphorus-containing vapor in the first reaction chamber, and the heating of the second reaction chamber, charging a reaction mixture of phosphate and reducing agent into the second reaction chamber wherein it is heated solely by contained heat of the walls thereof, and conducting the phosphorus-containing vapors evolved from the second reaction chamber to the first reaction chamber to be burned therein to supply heat therein for further reaction.

2. In the art of producing phosphorus, heating a mixture of phosphate mineral and coking coal to a coking temperature, thereby forming a reaction mixture of phosphate and carbonaceous material, preheating the interior walls of a reaction chamber to reaction temperature, then charging into said reaction chamber the reaction mixture, whereby it is heated therein solely by contained heat of the walls of the reaction chamber and the phosphate content of the reaction mixture is reduced and the resulting phosphorus evolved, conducting the resulting phosphorus to a second reaction chamber, burning it therein to heat its walls to reaction temperature, and thereupon supplying reaction mixture to the second reaction chamber for similar treatment therein.

3. In the art of producing phosphorus, the method which comprises heating a mixture of

phosphate rock and coking coal to a coking temperature, thereby producing a combustible hydrocarbon gas and a reaction mixture of phosphate and carbonaceous material, preheating a reaction chamber to reaction temperature, and thereupon charging said reaction mixture into the reaction chamber, whereby the reaction mixture is heated therein until it attains reaction temperature and to effect reaction with evolution of phosphorus-containing gases, conducting combustible hydrocarbon gases from the initial heating of the reaction mixture and coking coal into a second reaction chamber and burning them therein until the reaction mixture in the first reaction chamber begins evolving

phosphorus-containing gases, thereupon diverting said combustible hydrocarbon gases from the second reaction chamber and directing the phosphorus-containing gases from the first reaction chamber into the second reaction chamber and burning them therein, thereby preheating the second reaction chamber internally to reaction temperature, and thereupon discontinuing the heating of the second reaction chamber and introducing the reaction mixture of phosphate and carbonaceous material thereto, for reduction and evolution of its phosphorus content.

ARTHUR J. MASON. 15